

# UNITED STATES PATENT OFFICE.

JOHN H. STEVENS, OF NEWARK, NEW JERSEY, ASSIGNOR TO THE CELLULOID MANUFACTURING COMPANY, OF NEW YORK, N. Y.

## MANUFACTURE OF COMPOUNDS OF PYROXYLINE OR NITRO-CELLULOSE.

SPECIFICATION forming part of Letters Patent No. 269,345, dated December 19, 1882.

Application filed June 24, 1882. (No specimens.)

*To all whom it may concern:*

Be it known that I, JOHN H. STEVENS, of the city of Newark, in the county of Essex and State of New Jersey, have invented certain new and useful Improvements in the Manufacture of Compounds of Pyroxyline or Nitro-Cellulose, of which improvements the following is a specification.

It is well known to those skilled in this manufacture that alcohol is of itself a solvent of nitro-cellulose under certain conditions—that is to say, ordinary alcohol, (such as is known as "ninety-five per cent.") when heated to about 160° or 170° Farenheit, will readily dissolve the ordinary soluble forms of nitro-cellulose; or, if the nitro-cellulose is made extra soluble, it can be converted into a solid compound with ordinary alcohol by the use of heated rolls; or, again, with a sufficient quantity of absolute alcohol or dehydrated alcohol, the ordinary forms of soluble nitro-cellulose, such as are used in these compounds, can be readily converted in open rolls; but it is only with such qualifications that alcohol can be termed a "solvent of nitro-cellulose," and as the necessary conditions are difficult of attainment in the practical manufacture of these compounds alcohol alone is not used as a solvent, and, in a practical sense, is not classed with the solvents of pyroxyline. It is, however, a valuable ingredient of such compounds, and it is the object of my invention to render it available in the ordinary processes by employing in conjunction with it certain other ingredients, which, as I have discovered, when combined with ordinary alcohol, constitute or form solvents of nitro-cellulose under ordinary conditions.

It has long been known that, as above explained, while alcohol is not of itself an active or positive solvent of nitro-cellulose under ordinary conditions, yet in conjunction with camphor or with ether and with several other substances it forms such an active solvent. The category of these substances has heretofore been limited, and I have, by experiment, ascertained that while in themselves like alcohol

not solvents of pyroxyline, yet in conjunction with alcohol the following new menstrua constitute active solvents under ordinary conditions, to wit: acetal, nitrate of amyl, nitrite of amyl, oil of chamomile, oil of valerian, oil of golden-rod, oil of sassafras, oil of anise, light oil of cinnamon, oil of cumin, oil of cynæ ether, oil of dill, oil of elecampane, oil of fennel-seed, oil of eucalyptus, oil of fennel-chaff, oil of wine, (heavy,) oil of worm-seed, oil of myrtle, oil of laurel, oil of marjoram, oil of peppermint, oil of frue, oil of cinnamon-leaves, oil of palmarosa, oil of rosemary, (that from French flowers preferred.) oil of erigeron, and these are what I herein refer to as "new menstrua." The best practice in using these ingredients in conjunction with alcohol is to add the alcohol to the nitro-cellulose, incorporating in this mixture the coloring-matters and other inert substances to be included in the product, and then to add the new menstruum, which may be any one of those enumerated above, or a mixture of any two or more of them. The compound should be allowed to stand after the addition of the menstruum for about twelve hours in a closed vessel, and then be masticated in heated rolls in the usual manner, and the product should be formed into shapes before it has hardened or seasoned with time. Varying between the extremes given according as the menstruum selected is less or more volatile—the less volatile, as the oils, requiring the smaller proportion, and the more volatile, as the ethers, requiring the greater proportion—the proportions used will be about as follows: of pyroxyline, say, four parts, by weight; alcohol, three to four parts, by weight; any of the above-enumerated menstrua, (or mixtures of the same,) two to three parts, by weight.

Wood-spirit may be used in conjunction with alcohol and with my new menstrua; but in such case the menstruum should be first mixed with the nitro-cellulose and other ingredients, and the alcohol and wood-spirit mixed separately and added last. In other respects the treatment is the same as already described. With wood-spirit good proportions would be:

pyroxyline, two parts, by weight; alcohol, one part; menstruum, one part; wood-spirit, one part, all by weight.

Having thus described the nature and objects of my invention, what I claim as new, and desire to secure by Letters Patent, is—

As an improvement in the manufacture of compounds of pyroxyline, the employment, in

conjunction with alcohol, (ethylic or methylic,) of the hereinbefore-specified new menstrua or mixtures of the same, substantially as described.

JOHN H. STEVENS.

Witnesses:

ABRAHAM MANNERS,  
J. C. FORCE.